# EUROPEAN PATENT SPECIFICATION

(11) **EP 3 040 139 B1**
(45) Date of publication and mention of the grant of the patent: **25.07.2018**
(21) Application number: 15197388.0
(22) Date of filing: 01.12.2015
(51) Int. Cl.: B22D 17/00, B66B 21/00, C22C 21/00, C22C 21/06, C22C 21/08, B66B 23/12

(54) **USE OF AN ALUMINIUM ALLOY FOR AN ESCALATOR STEP OR AUTO-WALK PALLET AS A MECHANICAL PART**
VERWENDUNG EINER ALUMINIUMLEGIERUNG FÜR EINE ROLLTREPPENSTUFE ODER LAUFBANDSEGMENT ALS EIN MECHANISCHES TEIL
L'UTILISATION D'UN ALLIAGE D'ALUMINIUM POUR UNE MARCHE D'ESCALIER ROULANT OU POUR UNE PALETTE DE TROTTOIR ROULANT EN TANT QUE PIÈCE MÉCANIQUE

(30) Priority: 29.12.2014 CN 201410840662
(43) Date of publication of application: 06.07.2016
(73) Proprietor: Kone Corporation, 00330 Helsinki (FI)
(72) Inventor: Mäkimattila, Simo, 200051 Shanghai (CN)
(74) Representative: K & H Bonapat Patentanwälte Koch · von Behren & Partner mbB

(56) References cited:
- EP-A1- 1 477 577
- EP-A2- 0 940 564
- EP-A2- 1 178 125
- WO-A1-03/027345
- DE-A1- 4 336 037
- JP-A- H0 790 460
- JP-A- H0 820 833
- JP-A- H1 161 311
- JP-A- H1 161 312
- JP-A- H08 170 138
- JP-A- H11 293 375
- US-A1- 2002 006 352
- ASENSIO-LOZANO J ET AL: "Microstructure-properties correlation of pressure die cast eutectic aluminum-silicon alloys for escalator steps (Part II)", MATERIALS CHARACTERIZATION, ELSEVIER, NEW YORK, NY, US, vol. 56, no. 3, 1 April 2006 (2006-04-01), pages 178-184, XP027973840, ISSN: 1044-5803 [retrieved on 2006-04-01]

## Description

### Field of the Invention

The present invention relates to aluminum alloys, and particularly to aluminum alloys for use in manufacturing high-strength, light-weight die-cast escalator steps or auto-walk pallets.

### Background of the Invention

Current escalator steps or auto-walk pallets are manufactured via two distinctively different manufacturing routes, namely
a) High-pressure die-casting of aluminum alloys to produce a one-piece casting of full step body,
b) Fabricated, mechanical assembly of separate components of cold-rolled stainless steels, low-carbon cold-rolled sheet assembled with cast-iron and other metallic and polymer parts welded or mechanically joined to form a step body.

Document EP 1 178 125 A2 is related to the technical field of aluminum alloy sheets of the AlMg type and more particularly of the alloy 5083 or 5086 according to EN 573-3, intended not for die-cast but welded constructions such as fixed or mobile tanks and in particular tanks of road or rail transport of solid or liquid materials. This AlMg alloy sheet consists of in wt. %: 4.2-4.8 Mg; less than 0.5 Mn; less than 0.4 Zn; less than 0.45 Fe; less than 0.3 Si; and possibly less than 0.15 Cr; less than 0.25 Cu; less than 0.2 Ti; less than 0.2 Zr; other elements less than 0.05 each and less than 0.15 in total; balance Al with Mn+Zn less than 0.7.

Yield strength and tensile strength are two basic parameters widely used in engineering field. They are used for measuring the ability of metal materials to resist deformation and fracture under a loaded force. A die-cast aluminum alloy typically has yield strength up to 80-100 MPa but fractures at low total elongation of 1-2 %. Due to the low strength and brittle fracture behavior of die-cast aluminum alloy, die-cast aluminum alloy steps are likely to break during service, and thus lead to risk of passenger injury.

Strength/weight ratio is another parameter to evaluate the performance of metal materials, which is the ratio between tensile strength and apparent density. A higher strength/weight ratio indicates that less mass of the material is required to reach a determined strength. So far the known attempts to improve strength/weight ratio of escalator step or auto-walk pallet castings are as follows:
- Improve the strength of aluminum-silicon alloy. Aluminum-silicon alloys (8-13% Si) are the most extensively used alloys in die-casting. Thyssen-Krupp has published studies to use rare-earth metals (as grain refiner during solidification) to produce an aluminum-silicon casting alloy material with improved properties. The resulting strength of silicon alloy material is lower than that of aluminum-magnesium alloys if used with current casting practice. The resulting ductility of silicon alloy material has not been observed to be improved.
- Use high strength steel materials in combination with aluminum alloy materials, to achieve a safe and ductile behavior of the resulting escalator step or auto-walk pallet castings. This approach requires a long assembly process, and involves joining processes as well. Separate joining parts are costly in terms of, for instance, the associated labor and inspection, intermediate finishing and individual part fabrication.
- Thyssen has published escalator steps made from fiber-reinforced plastics as a low-weight, less-noise solution. However material cost, production cost and fire-resistance may appear problems of implementation.
- Automotive industry has developed aluminum-magnesium cast alloys for automotive body parts, shock absorber supports and wheel suspension parts because of energy-efficiency, fuel-efficiency and material saving.

### Object and Summary of the Invention

The present invention is directed to the use of an aluminum alloy as the mechanical parts in a high-strength, light-weight die-cast escalator step or auto-walk pallet.

The aluminum alloy according to the present invention consists of:
4 to 6 % by weight of magnesium;
0.3 to 0.9 % by weight of ferrum;
0.1 to 0.6 % by weight of manganese; and
0.2 to 2 % by weight of silicon, with the remaining rest being aluminum.
It has been observed that the aluminum alloy of the present invention has achieved higher strength, higher ductility and lower weight, as compared with existing aluminum alloys.

According to the invention, a mechanical part made from the aluminum alloy according to the present invention is provided. Specifically, the mechanical part is an escalator step, or an auto-walk pallet.

It has been observed that the resulting escalator step or auto-walk pallet exhibited excellent performances including, but not limited to, lower weight, higher strength, and higher total elongation, as compared with the current escalator step or auto-walk pallet.

According to the invention, use of the aluminum alloy according to the present invention is provided. By virtue of the enhanced performance, the aluminum alloy according to the present invention is suitable for use in manufacturing mechanical parts, especially for those are required to constantly or frequently withstand a high loaded force, such as mechanical parts of escalator steps or auto-walk pallets.

### Detailed Description

Reference will now be made to an embodiment of the disclosure. The embodiment is provided by way of explanation of the disclosure, and is not meant as a limitation of the disclosure. It is intended that the disclosure encompass these and other modifications and variations as come within the scope of the disclosure.

According to one embodiment of the present invention, the aluminum alloy of the disclosure consists of 4 to 6 % by weight of magnesium; 0.3 to 0.9 % by weight of ferrum; 0.1 to 0.6 % by weight of manganese; and 0.2 to 2 % by weight of silicon, with the remaining rest being aluminum. One of ordinary skill in the art should understand that the aluminum alloy of the disclosure may comprise unavoidable impurities.

The aluminum alloy of the present invention has the required strength and higher fatigue strength to enable weight reduction.

The aluminum alloy of the present invention is suitable for use in manufacturing mechanical parts. Specifically, the aluminum alloy may be cast into the thin-walled escalator step or the auto-walk pallet. The resulting escalator step or auto-walk pallet has yield strength of 160 MPa and high ductility of 16 % against step/pallet break. Furthermore, the escalator step or auto-walk pallet of the present invention meets the step/pallet ultimate breaking test load at lower step/pallet weight level, 15-20 %, due to the lower material specific weight and the smaller cross-sectional area of the load carrying members.

The aluminum alloy of the present invention can be cast into a thin-wall thickness of 1.0-1.2 mm at minimum, by using tools according to the state-of-art, such as steel molds and dies, and by using currently known casting practices. The step cross section dimensions required by a normal cast step can be achieved with lower specific weight, higher strength and higher total elongation, which is more safe for escalator passenger in case of step breaking due to escalator misuse, unexceptional loading of step due to mechanical failure of other components, such as falling of foreign objects on step band, mechanical material fatigue, wear, aging and corrosion.

Escalators and auto-walks have several safety devices to prevent injury due to step crash. Step crash may occur due to mechanical failure of the guiding parts, chain, chain guide, step roller, drive chain or any dislocation, chain break, wear and misuse. In case of such crash the advantage of high-strength ductile material is that it does not break in brittle way but deforms preventing passenger fall.

Auto-walks operate in horizontal direction where the lower step weight contributes to lower power consumption because of reduction of moving masses vs passenger load and the associated lower friction force.

The die-cast escalator step or auto-walk pallet of the disclosure has the structural design and material properties as defined by the industry prior art as well as international codes and norms:
- load forces determined by the step area where passengers can stand, 6000 N/m2, including additional strength due to safety factor of 3-4;
- fatigue resistance up to 6 million load cycles;
- corrosion resistance against road salt, marine climate;
- friction coefficient against passenger footwear to prevent falling due to slippery, especially when escalator/auto-walk stops via safety devices activation;
- corrosion resistance for outdoor use, in public transport facilities like metro stations, airports, against direct rainfall in marine climate;
- corrosion resistance due to road salt in climatic zones of seasonal sub-zero temperatures for outdoor and indoor use;
- thread design to allow smooth conduction of passenger over comb area;
- wear resistance to keep the comb safety gap;
- wear and dimensional stability (castability) to keep the skirting gap and comb gap safety function.

It should be noted that the above described embodiment is given for describing rather than limiting the invention, and it is to be understood that modifications and variations may be resorted to without departing from the spirit and scope of the invention as those skilled in the art readily understand. Such modifications and variations are considered to be within the scope of the invention and the appended claims. The protection scope of the invention is defined by the accompanying claims.

## Claims

1. Use of an aluminum alloy consisting of:
4 to 6 % by weight of magnesium;
0.3 to 0.9 % by weight of ferrum;
0.1 to 0.6 % by weight of manganese; and
0.2 to 2 % by weight of silicon,
with the remaining rest being aluminum, for producing an escalator step or auto-walk pallet as a mechanical part, wherein the escalator step or autowalk pallet is made by die-casting.

## Patentansprüche

1. Verwendung einer Aluminiumlegierung, die besteht aus:
4 bis 6 Gewichtsprozent Magnesium;
0,3 bis 0,9 Gewichtsprozent Eisen;
0,1 bis 0,6 Gewichtsprozent Mangan; und
0,2 bis 2 Gewichtsprozent Silizium,
wobei der verbleibende Rest Aluminium ist, zum Herstellen einer Fahrtreppenstufe oder Rollsteigpalette als einem mechanischen Teil, wobei die Fahrtreppenstufe oder Rollsteigpalette durch Druckgießen gefertigt wird.

## Revendications

1. Utilisation d'un alliage d'aluminium, composé de :
4 à 6 % en poids de magnésium ;
0,3 à 0,9 % en poids de fer ;
0,1 à 0,6 % en poids de manganèse ; et
0,2 à 2 % en poids de silicium,
le reste étant de l'aluminium, pour la production d'une marche d'escalier mécanique ou d'une palette de trottoir roulant en tant que pièce mécanique, dans lequel la marche d'escalier mécanique ou la palette de trottoir roulant est réalisée par moulage mécanique.
